

J. SLATTERY.

PROCESS OF AND APPARATUS FOR FORMING COMPOUND INGOTS.  
APPLICATION FILED JAN. 5, 1915.

1,172,747.

Patented Feb. 22, 1916.

3 SHEETS—SHEET 1.



Witnesses:

Misses.  
Mrs. B. A. Doring  
Paul H. Franke

### Inventor

John Slatery

By his Attorneys *Marshall & Slaty*

J. SLATTERY,

PROCESS OF AND APPARATUS FOR FORMING COMPOUND INGOTS.  
APPLICATION FILED JAN. 5, 1915.

1,172,747.

Patented Feb. 22, 1916.

3 SHEETS—SHEET 2.



Witnesses:

Mass.  
Haze B. A. Doring  
Paul H. Franke

**Inventor**

John Slattery

By his Attorneys  
Marbler & Matty

J. SLATTERY.

PROCESS OF AND APPARATUS FOR FORMING COMPOUND INGOTS.

APPLICATION FILED JAN. 5, 1915.

1,172,747.

Patented Feb. 22, 1916.

3 SHEETS—SHEET 3.



# UNITED STATES PATENT OFFICE.

JOHN SLATTERY, OF CHROME, NEW JERSEY.

## PROCESS OF AND APPARATUS FOR FORMING COMPOUND INGOTS.

1,172,747.

Specification of Letters Patent.

Patented Feb. 22, 1916.

Application filed January 5, 1915. Serial No. 554.

To all whom it may concern:

Be it known that I, JOHN SLATTERY, citizen of the United States of America, and a resident of Chrome, county of Middlesex, 5 and State of New Jersey, have invented certain new and useful Improvements in Processes of and Apparatus for Forming Compound Ingots, of which the following is a specification.

10 My invention relates to processes and apparatus for forming compound ingots, particularly ingots composed of layers of low carbon and high carbon steel, united; and the invention pertains particularly to that 15 class of such processes and apparatus wherein a septum is provided, within the ingot mold, which septum, without absolutely preventing contact of the two grades of molten metal, retards the flow of the two 20 metals toward each other to such extent that the metals unite with very little mixing. The septum is commonly of metal, of a melting point and nature such that it will be melted by the molten metal and so will 25 be incorporated practically indistinguishably into the metal of the resulting compound ingot.

While such processes have been proposed heretofore, yet so far as I am informed, 30 practical difficulties have prevented their use, at least to any considerable extent, and particularly in the formation of large ingots such as are required in the production of armor plate, rail steel, vault or safe steel, 35 rolling mill rolls, etc. These practical difficulties are overcome by the process and apparatus herein described.

According to one method of carrying out my invention the septum employed is, preferably, a structure composed of a series of plates hung vertically within the mold in such manner as to provide staggered openings for the flow of the two metals together, the tortuous nature of the passages formed 45 by these staggered openings sufficing to so retard the flow of the metals toward each other to such extent that the metals unite in the molten state with very little mixing, the septum becoming incorporated with the 50 said metals as they solidify. But other constructions of septa presenting staggered openings for the flow of the two metals together may be employed without departing from my invention, and I do not limit my-

self to the use of septa presenting tortuous 55 passages for the flow of the molten metals toward each other.

That side of the mold which is to receive the high carbon steel is preferably provided with a runner or runners of refractory material, such as fire brick, extending from near the bottom of the mold upward, and having lateral openings for the flow of the molten metal into the mold; this construction being employed to prevent the very 60 fluid high carbon steel from melting down the septum prematurely, and from melting down the sides of the mold. Both sides of the mold may be provided with such runners, but in general it is not necessary to 65 provide the low carbon steel side of the mold with such a runner with lateral openings. I prefer to pour the low carbon steel side of the mold from the top, using a head box to control and direct the flow of the 70 molten metal, and preferably I also employ a similar head box for the supply of molten high carbon steel to the said runner for the high carbon steel side of the mold, regulating the flow of the steel through these head 75 boxes so that the molten metals are kept at approximately equal heights on the two sides of the septum during the pouring. In this way, the incoming hot metal is kept at the top of the body of molten metal, in 80 each chamber of the mold; something of very great importance; the ingot therefore begins to cool first at the bottom, the cooling progressing upwardly gradually, the 85 septum retaining its integrity (since it requires an appreciable time to melt it) until the molten metal is pasty, or nearly so. This manner of pouring the ingot, i. e., pouring it in such manner that the incoming hot metal overlies the colder metal already within the mold, tends to prevent 90 piping in the ingot, since the more fluid metal above tends to fill any pipe formed below. These matters will be explained at greater length hereinafter. 100

My invention consists in the novel process of forming compound metal ingots, comprising the flow of both bodies of molten metal into the mold from the top, and the regulation of the rate of flow with reference to the rate of melting of the septum; in the combination of an ingot mold having a septum and pouring heads; in an ingot

mold having on one side a runner with lateral openings into the mold; in the construction of the septum, and in various other features all as hereinafter described and particularly pointed out in the appended claims.

In the accompanying drawings I illustrate more or less diagrammatically, apparatus which may be employed in carrying out my invention.

10 In said drawings, Figure 1 shows a side elevation of an ingot mold, and head boxes therefor, all constructed in accordance with the apparatus portion of my invention, and adapted for carrying out the process portion of my invention. Fig. 2 shows a top view of the mold itself, and of the septum therein. Fig. 3 shows a vertical section of the ingot mold on the line  $x-x$  of Fig. 2, and also shows the head boxes above the 15 mold, one of these head boxes being shown in section. Fig. 4 shows a vertical section of the ingot mold and head boxes on the line  $y-y$  of Fig. 2. Fig. 5 shows a vertical section of an alternative form of mold, having 20 a runner with lateral openings for each of the two bodies of molten metal. Fig. 6 shows a top view of an ingot mold of generally circular form, and illustrates the application of my invention to the formation 25 of combined ingots wherein one grade of metal surrounds the other grade of metal.

In the drawings numeral 1 designates the ingot mold, 2 a floor plate upon which the same may rest, 3 a removable mold top, 4 a lateral extension of the mold to receive the sectional runner 5, and 6 the septum, composed in the main of a series of staggered plates  $6^a$ , as indicated particularly in Fig. 2. Suitable means, such for example, as cleats 40 7 provided on the floor plate 2, and wedges 8 adapted to be driven between the mold and these cleats, are provided for holding the mold in place on the floor plate. Suitable means, such for example as wedges 9 secured to the mold top 3 and adapted to fit 45 between lugs 10 on the sides of the mold, are provided for centering the mold top with reference to the mold; and suitable means, such as yokes 11 and wedges 12 engaging 50 lugs 13 on the sides of the mold and mold top, are provided for holding the mold top in place. The details of construction of these parts are familiar and require no further mention.

55 As previously stated, the septum is composed in the main of staggered plates  $6^a$ , these plates being held in proper relative relation by slotted plates  $6^b$  in the slots of which plates  $6^b$ , the vertical plates  $6^a$  are held tightly, as by close frictional engagement. Suitable means may be provided for holding the septum 6 down; i.e., for preventing it from flowing in the molten metal. To this end I have indicated the mold top 60 3 as provided with an internal flange 14

which will rest upon the top of the uppermost plate  $6^b$ , pressing the septum down with sufficient firmness to prevent that septum from being displaced by surging of the molten metal against it.

70 The refractory runner 5 is formed in sections  $5^a$ , as shown particularly in Fig. 3; these sections having registering central passages 15 and lateral orifices 16 leading into the interior of the mold, these orifices being 75 staggered preferably, as indicated in Fig. 4. By making each of these openings 16 of relatively small height, and staggering them, I provide ample strength for the runner sections  $5^a$ , without interrupting in any 80 way the continuous flow of the molten metal from the runner into the mold.

85 As heretofore stated by me, various plans have been proposed heretofore for the formation of combined ingots by pouring molten metal of different grades on opposite sides of a septum; but, so far as I am informed, without success, at least where the formation of large ingots of metal of such high melting point as steel is concerned. 90 According to one such method, the ingot mold is to be divided by two perforated partitions, set into the mold, and spaced somewhat apart one from the other, means being provided for running molten metal 95 from below into the mold on the two sides of the double partition thus formed. According to my experience, this method of forming compound ingots cannot be successfully carried out, at least when the septum is intended to melt and become incorporated 100 with the cast metal, for since the molten metal enters the mold from below, the first metal that comes into the mold stays on top, rising as more molten metal enters the 105 mold. The result must be, inevitably, that the septum plates will be melted away in the lower part of the mold only, the remainder of the septum plates not being melted at all, and probably, not combining 110 at all with the cast metal; while, on the other hand, the lower portions of these septum plates will be melted so quickly that the two incoming streams of hot metal will mingle greatly, thus defeating the purpose 115 for which the septum is used. According to my experience, such a method as that referred to must necessarily result in an ingot of very ununiform quality, an ingot in which the two grades of metal are mingled 120 indistinguishably in the lower part, while in the upper part of the ingot the two grades of metal will probably not be united at all. Moreover, since in the old proposed method referred to, the metal first poured rises, being replaced continually by fresh hot metal beneath, piping is very apt to start in the 125 top of the ingot without any material tendency toward the filling of pipes, if formed, by the more fluid metal beneath; and fur-

130

thermore, the upper metal of the ingot is apt to shrink away from the sides of the mold.

According to another formerly proposed method, the mold is to be divided internally by two imperforate plates spaced apart, and, apparently, of sufficient thickness to resist fusion by the molten metal lying against them until the mold is substantially filled; at which time the partition plates mentioned are supposed to melt down permitting the two grades of molten metal to flow together. It is not stated how the mold is to be poured, *i. e.*, whether from above or from below. Obviously it would be very difficult to provide dividing plates of just the right material and just the right thickness to resist the fusing tendency of the molten metal until the mold is practically full, and then to melt down with sufficient rapidity throughout their length to permit substantial uniform union of the two molten metals while those metals are still hot enough to unite, and yet not so fluid as to become mingled indistinguishably. In fact, such a method forms, artificially, an exaggerated "pipe"; just what is most to be avoided. It is impossible to believe that by such a method, compound steel ingots could be produced in which the two grades of steel are united with substantial uniformity throughout the length of the ingot, and without being mixed to such an extent that there could hardly be any difference between the metal on one side of the ingot and the metal on the other.

Now according to my invention the mold is poured, on both sides of the septum, from the top, but in such manner that the molten metals are prevented from washing down along the sides of the ingot mold and of the septum, and thereby are prevented from cutting the sides of the ingot mold and from melting the septum prematurely. To the contrary, the molten metal enters the mold somewhat quietly, the lower carbon steel, in particular, entering the mold in a solid stream, which spreads out, the metal which first enters the mold remaining at the bottom of the mold, each increment of the molten metal remaining substantially at the level at which it encounters the molten metal already within the mold. Of course, the two molten metals pass through the tortuous passages of the septum and contact one with the other, as is intended. But the resistance offered by these tortuous passages to the flow of the molten metal is such that no considerable mixture of the two grades of metal with each other occurs. The metals which first enter the mold soon melt down the portions of the septum plates immersed in such metals; but by the time this has occurred the molten metal, up to the level at which the melting occurs, has become relatively quiet,

and moreover has already begun to solidify, at least to the extent of becoming pasty, and so little or no mixing of the two grades of metal occurs; and this action progresses upward along the septum as the mold is filled; the septum resisting the tendency of the molten metal to flow together and mix for a time, and then, as the septum is melted, permitting the two metals to unite, but only when they have become so thick as not to become diffused one within the other. Obviously, for success with this method of forming ingots, some control of the rate at which the molten metal is introduced is required, and for this purpose head boxes, or pouring boxes, 17 and 18 are provided. They are provided with bottom openings 19 and 20 respectively, through which the molten metal within them passes down into the ingot mold. The discharge opening 19 of the pouring box 17, used for the lower carbon steel, is preferably provided with a spout 21 of such length as may be found most suitable for the particular grade of steel and size of the ingot to be made. Such an elongated opening 19 gives to the downwardly directed stream of molten metal, the characteristic of a solid stream, as distinguished from a spray stream; and thereby the molten metal is prevented from spreading out, before it reaches the top of the molten metal already in the ingot mold, and so is prevented from washing down the sides of the ingot mold and of the septum; furthermore, being in a solid stream, it retains its heat much better, and is less affected by the air. Proper regulation of the rate of flow of the molten metals may be obtained by regulating the height to which the pouring boxes are kept filled during the progress of the pouring; and by regulating the size or diameter of the openings 19 and 20; and of course, it is practicable for the attendants to obstruct the openings 19 and 20 temporarily by clay plugs or the like, in the well known manner, if further restriction is required.

In general, it is unnecessary to provide pouring head 18 for the high carbon steel with a spout such as the spout 21 of the pouring head 17, for the reason that the pouring head 18 may be located a short distance only above the runner 5, and that runner itself prevents the molten metal from spreading out, and forces it to enter the mold quietly. The pouring head 17 may be suspended from above, and its spout 21 may be of such length that such spout will be well within the mold, when the pouring is started, the molten metal then having only a short distance to fall; and as the level of the molten metal rises in the mold the pouring head 17 may be raised. To prevent the floor plate from being eaten away by the molten metal entering through pouring head 17, a body 22 of refractory material may be provided

in this floor plate to receive the impact of the first of the molten metal. This refractory body 22 is, of course, renewable. However, and as indicated particularly in Fig. 5, runners 5 may be provided on both sides of the septum.

The inside of the mold top 3 is protected, preferably, by a covering 23 of sand or fire clay or the like.

10 Not only is the septum herein illustrated and described relatively cheap and easy to make, but it is the first septum of which I am aware, in which adequate provision is made for expansion of the septum itself, 15 with rise of temperature without disturbance of the position of the septum in the mold, and without warping of the septum. While the spacers 6<sup>b</sup> hold the septum plates 6<sup>a</sup> quite firmly, yet extension of the plates 20 6<sup>a</sup> through the holes of the upper spacer 6<sup>b</sup> is permitted, this upper plate 6<sup>b</sup> being held in place by the flange 14 of the mold top 3.

My invention is not restricted to the formation of rectangular ingots. It is equally 25 applicable to the formation of ingots of circular or other non-rectangular cross section.

In Fig. 6 I show an ingot mold of a corrugated exterior contour, the general form of the ingot being cylindrical. 6<sup>a</sup> designates 30 the septum, and 5' runners for the mold similar to the runner 5 of Figs. 1-4 inclusive. 6<sup>a</sup>' designates the staggered plates of the septum and 6<sup>b</sup>' the slotted plates holding plates 6<sup>a</sup>' in place.

35 From what has been said above, it will be clear that not only will this process produce combined ingots of substantially uniform quality from one end to the other, and with perfect union obtained between the two 40 grades of metals without material diffusion of one metal into the other, but also that there is relatively little tendency toward piping, as compared with ingots formed in other ways; for, since the metal poured 45 first solidifies first, and in the lower portion of the mold, the still highly fluid metal above tends to flow down into and fill any pipes formed in the solidifying metal below.

What I claim is:—

50 1. The herein described method of casting compound metal ingots, which consists in flowing molten metal from different sources, into a suitable mold on opposite sides of a septum dividing that mold, each stream of 55 molten metal entering the mold from above and in the form of a quiet stream which spreads out with little disturbance of the molten metal beneath, each increment of the molten metal remaining substantially at the 60 level at which it encounters the molten metal already within the mold, and by the heat of the molten metal melting the septum upward progressively and causing its material to combine with the cast metal, and 65 regulating the flow of both streams of

molten metal with reference to the rate of melting of the septum to preserve substantial integrity of each portion of the septum until the molten metal in contact with such portion has cooled to such extent that little 70 diffusion of the two bodies of molten metal in one another will occur upon the melting of that portion of the septum.

2. The herein described method of casting compound metal ingots, which consists 75 in flowing molten metal from different sources into a suitable mold on opposite sides of a septum dividing that mold, but affording restricted passages for contact of the two bodies of molten metal with one 80 another, both streams of molten metal entering the mold from above, and mingling to some extent by passage through the restricted passages of the septum, and by the heat of the molten metal melting the septum 85 upward progressively and causing its material to combine with the cast metal, and regulating the flow of both streams of molten metal with reference to the rate of melting of the septum to preserve substantial 90 integrity of each portion of the septum until the molten metal in contact with such portion has cooled to such extent that little diffusion of the two bodies of molten metal in one another will occur upon the melting 95 of that portion of the septum.

3. Apparatus for forming compound metal ingots comprising an ingot mold having a septum dividing its interior, in combination with means for introducing molten metal of different grades into the mold on opposite sides of said septum, both of such molten metal supply means comprising means for delivering the molten metal into the mold from above and for delivering 100 such molten metals in quiet streams.

4. Apparatus for forming compound metal ingots comprising an ingot mold having a septum dividing its interior, in combination with pouring heads having bottom 110 openings adapted to discharge two different bodies of molten metal, at least one of them in the form of a quiet stream into said ingot mold on opposite sides of said septum and not directed thereagainst.

5. Apparatus for forming compound metal ingots comprising an ingot mold having a septum dividing its interior, in combination with means for introducing molten metal of different grades into the mold from above on opposite sides of said septum and not directed thereagainst, one of said molten metal introducing means being a pouring head having a bottom spout.

6. Apparatus for forming compound metal ingots comprising an ingot mold having a septum dividing its interior, and having, on one side of said septum, a runner having a longitudinal passage with lateral flow means leading from such longitudinal 125 130

passages into the mold, such lateral flow means extending continuously from near the bottom of the mold to near the top thereof.

5 7. Apparatus for forming compound metal ingots comprising an ingot mold having a septum dividing its interior, and having, on one side of said septum, a runner having a longitudinal passage with a series 10 of lateral staggered openings leading from such passage to the mold, such series of openings extending from near the bottom of the mold to near the top thereof.

8. An ingot mold having on one side a 15 runner having a longitudinal passage with a series of lateral staggered openings leading from such passage to the mold, such series of openings extending from near the bottom of the mold to near the top thereof.

20 9. A mold septum comprising bodies arranged in a plurality of rows, the bodies in each row separated one from another and the bodies of one row opposite the spaces between the bodies of another row, in combination with means holding such bodies in 25 such spaced arrangement.

10. A mold septum comprising bodies arranged in a plurality of rows, the bodies in each row separated one from another and 30 the bodies of one row opposite the spaces between the bodies of another row, in combination with means holding such bodies in such spaced arrangement, and affording opportunity for longitudinal expansion of 35 said bodies.

11. A mold septum comprising a plurality of bodies spaced apart one from another, in combination with spacing means therefor, comprising a spacing member having openings through which such bodies pass, such spacing member adapted to permit longitudinal expansion of said members.

40 12. The combination with an ingot mold of a septum therein having a plurality of

tortuous passages through it for the flow of 45 molten metal.

13. The combination with an ingot mold, of a septum therein comprising a plurality of bodies spaced one from another, spacing means for said bodies and a mold top having 50 means engaging said spacing means and thereby holding the septum in place.

14. The combination with an ingot mold, of a septum therein comprising a plurality of bodies spaced one from another, spacing 55 means for said bodies and a mold top having an inwardly projecting flange engaging said spacing means and thereby holding the septum in place.

15. Apparatus for forming compound 60 metal ingots comprising an ingot mold having a septum dividing its interior, in combination with means for flowing molten metal from different sources into said mold on opposite sides of said septum, and not 65 directed thereagainst, and for supplying such molten metal progressively to the top of molten metal already within the mold, such molten metal supply means comprising means for restricting the rate of flow of 70 molten metal into the mold.

16. Apparatus for forming compound metal ingots comprising an ingot mold having a septum dividing its interior, in combination with means for introducing molten 75 metal of different grades into the mold on opposite sides of said septum and not directed thereagainst, said molten metal supply means each comprising means affording a substantially constant rate of flow of the 80 molten metal into the mold.

In testimony whereof I have signed this specification in the presence of two subscribing witnesses.

JOHN SLATTERY.

Witnesses:

H. M. MARBLE,  
PAUL H. FRANKE.